

## UNITED STATES PATENT OFFICE

1,966,821

## GREASE AND ITS MANUFACTURE

Gus Kaufman, Beacon, N. Y., assignor to The Texas Company, New York, N. Y., a corporation of Delaware

No Drawing. Application August 15, 1931,  
Serial No. 557,385

4 Claims. (Cl. 87—9)

This application is a continuation-in-part of my copending application filed July 1, 1930, Serial No. 465,144.

This invention comprises a method of heat treating oils used in the preparation of lubricating greases, and particularly heat treating a mixture of a mineral oil and a soap forming material, such as a fatty oil, fatty acid and the like. The invention also has reference to the preparation of lubricating greases having a hardness or penetration especially adapting them for use as lubricants for driving journals of locomotives and having a relatively low soap content and relatively high mineral oil content.

Broadly, my invention contemplates the preparation of grease or lubricating compositions composed mainly of hydrocarbon oil and a soap prepared and combined in such a manner that the physical properties of the resulting grease, such as melting point and hardness, may be varied to a considerable extent substantially independently of the soap content.

The invention contemplates an improved method of manufacture of grease compositions wherein the hydrocarbon oil and fatty oil ingredients are preliminarily heated, preferably in admixture, under various conditions of temperature or during various periods of time at various temperatures in order to effect a digestion or conversion. The extent of this conversion may conveniently be controlled by regulating the increase in viscosity to a predetermined point. When the desired extent of conversion has been effected, alkaline material is added to react with the saponifiable constituents of the digested oil mixture to form a final product of desired physical and chemical characteristics.

It has been common in the prior grease making art to heat the mineral oil or hydrocarbon and fat or fatty acid together to the desired temperature for carrying out saponification, which might have been in some instances as high as 400 to 500° F. The aqueous solution of saponifying agent was then added without further delay in such regulated quantities that the water would be flashed off continuously, thus avoiding the possibilities of boil-overs due to excessive foaming. The time of manufacture of a batch was also materially reduced by this method.

According to the present invention the min-

eral oil and fat or fatty acid are not only heated together to a high temperature but they are maintained at a high temperature for a substantial period during which the aforementioned increase in viscosity occurs. In the light of the prior art method this heating may be said to be "needlessly" prolonged.

The physical and chemical properties of greases made according to the methods of the prior art are largely dependent upon the nature of the ingredients used in their preparation. Thus it has been customary, for example, to control the hardness of grease by varying the soap content, the hardness of the grease as commonly prepared usually being roughly directly proportional to its soap content.

Even when very high melting point or high titer fats are employed in the preparation of a hard grease by the prior art methods, the soap content of the resulting product may very greatly exceed that of my product having the same hardness and prepared from lower melting point fats.

By following the method of my invention an improved grease is produced, certain of the characteristics of which may be varied at will, but generally speaking one which has a melting point appreciably lower than that of grease of corresponding hardness manufactured by conventional methods of practice from substantially similar type ingredients. Greases made by employing my invention may contain materially lower proportions of soap than greases prepared by the prior art methods. In other words, if it is desired to produce a grease having a certain consistency or hardness the soap content necessary to attain such consistency or hardness may be reduced to any desired extent up to 30 to 50% less soap, and in some instances considerably greater reduction by the use of my invention. As a consequence of this the resultant grease will contain a larger proportion of hydrocarbon or lubricating oil, thus tending not only to very materially increase the lubricating qualities but also to greatly reduce the cost, inasmuch as a portion of the more expensive soap ingredient will have been replaced by the less expensive mineral oil ingredient.

Likewise it has been found that lower viscosity lubricating oils may partially or wholly replace higher viscosity lubricating oils in the preparation

of greases by my method, while attaining the same consistency or hardness as when using the more viscous oils. By the substitution of lower viscosity oils for higher viscosity oils while maintaining a given consistency or hardness, considerable advantages have been experienced in reducing the frictional resistance on account of the presence of the lower viscosity lubricating oil.

Notably in the case of greases employed in the lubrication of driving journals of locomotives, it is necessary generally to provide a grease which is very hard as compared with greases employed on other types of machinery. Such locomotive driving journal lubricants manufactured by the methods of the prior art commonly contain between 40% and 50% of the sodium soap of a high melting point fatty acid, or equivalent fat, this high percentage of soap having been found necessary to attain the desired hardness in the finished grease. These prior art driving journal lubricants commonly have a high melting point of about 450° F. On the other hand, a similarly hard grease for driving journal lubrication may be prepared according to my invention from similar ingredients with a soap content lower than 40%, and which soap content may vary even to as low as 20 to 25%. The grease prepared according to this invention may therefore contain a correspondingly larger proportion of mineral oil and may on this account have very superior lubricating qualities.

Such a low soap content and relatively high oil content grease has been found to be especially adapted to the very severe conditions present in locomotive driving journal lubrication. Furthermore, such grease may have a melting point of 350 to 400° F., which is considerably lower than that of the prior art greases, as pointed out above. The relatively low melting point is believed to be a distinct advantage in the lubrication of locomotive driving journals, since the grease tends to soften and feed onto the bearing surface at a lower bearing temperature, and generally tends to maintain the journal at a lower operating temperature than is the case with the usual driving journal grease.

So far as I am aware, the commercial driving journal compounds of the prior art have been prepared solely with cylinder oils or cylinder stock as the mineral oil constituent. Heretofore it has been deemed necessary to use a heavy mineral oil of that character to furnish the proper lubrication for such heavy duty journals, and also to attain the desired hardness of the driving journal grease. However, I am enabled by my invention to produce a locomotive driving journal lubricant of the usual hardness, characterized not only by the fact that the soap content may be exceptionally low, as pointed out above, but also by the fact that lower viscosity mineral oils, or at least a blend of cylinder stock and substantial amounts of lower viscosity oils, may be used. This may account in whole or in part for the fact that lower bearing temperatures obtain in the use of driving journal greases prepared according to my invention, perhaps because of the lower frictional resistance of the lower viscosity mineral oils compared with cylinder stock. In any event, it has been the experience in large scale practical use of such greases that they develop appreciably lower journal temperatures, and the lubrication furnished is uniformly superior to that of the prior art greases.

Broadly speaking, my invention contemplates the preparation of lubricating compositions or

greases, having desired lubricating and other physical properties, which may be composed of mineral and fatty oil or fatty acid ingredients of varying nature and physical characteristics and wherein the physical properties of the final product, particularly its consistency or hardness, may substantially be controlled irrespective of either its soap content or of the particular type of mineral or fatty oil used in its preparation. The petroleum or hydrocarbon lubricating oil constituents may be of the nature of a cylinder oil or cylinder stock and may embrace either a distillate or a residual product derived from either paraffin or naphthene base, or mixed paraffin and naphthene base crudes, or, on the other hand, may be of the nature of a pale oil or a fraction of lower boiling range than cylinder oil though derived from any of the foregoing crude sources. The fatty oil or fatty acid may be derived from either animal or vegetable origin, such as hard tallow, tallow oil, fleshing grease, stearin, elaine oil, castor oil, cottonseed oil, residual pitchy material resulting from the destructive distillation of fatty oils and fatty acids, and the like, and may also embrace hydrogenated fats.

The general procedure followed in preparing lubricating compositions in accordance with my invention is as follows: The hydrocarbon or mineral lubricating oil and fatty oil ingredients are mixed in suitable proportion, depending upon the quantity of these ingredients desired in the final product and are heated to a desired digestion or conversion temperature. During this heat treatment the oils are preferably continuously stirred. This temperature of treatment may range from approximately the melting point of the resulting grease, as for example 400° F., or even lower, to upwards of 600° F. The heated mixture of oils is then maintained substantially constant at the desired temperature for a predetermined period of time or until the mixture attains a desired degree of digestion or conversion, preferably determined by a progressive increase in the viscosity of the admixture. The digested mixture is then saponified in the usual manner by addition thereto of a suitable alkaline material such as caustic soda, lime, or the like, either with or without prior cooling of the digested mixture.

Although it is usually preferable to subject the petroleum and fatty oil ingredients to heat treatment after mixing, it is contemplated that these ingredients may be separately subjected to heating or digestion with subsequent mixing while in a heated state prior to saponification for the production of certain lubricating compositions.

While the exact nature of the physical and chemical changes occurring during digestion of the mixture has not been determined, apparently certain new compounds or products of reaction are formed which impart desirable qualities, especially that of hardness, to the resulting final product and which may be formed as the result of reaction during digestion or conversion, between the mineral and fatty oil, between constituents thereof, or between compounds or products formed as a result of conversion or partial decomposition of the fatty and mineral oils during the heat treatment or as the result of a combination of such reactions. These reactions may result in part at least from oxidation of the hot mixture resulting from the contact of the atmosphere with the surface of the mixture, or the mechanical stirring into the mixture of some of the air over it. This theory is strengthened by reason of the fact that it has been found that

80

85

90

95

100

110

115

120

125

130

135

140

145

150

the desired increase in viscosity, and resulting increase in the hardness of the final grease, is hastened somewhat by the introduction of air into the mixture.

5 These reactions are usually accompanied by corresponding and progressive changes in the physical characteristics of the mixture during digestion, such as discoloration and increasing viscosity, so that the duration of heat treatment 10 may readily be controlled by observation of these progressive physical changes and is preferably determined by the change in viscosity of the digesting mixture.

15 The oil mixture is preferably heated to the desired digestion or reaction temperature as rapidly as possible in a conventional type grease kettle, after which it may be maintained substantially constant at the desired temperature by controlling the rate of firing the furnace until the mixture 20 has attained a predetermined viscosity. It is desirable to effect more or less constant agitation of the mixture. Thus the mixture may be raised to a relatively low temperature, for example from 400° F. to 480° F., and be maintained at substantially this temperature for a relatively 25 long period of time, while on the other hand the oil may be heated to a relatively higher temperature, ranging from 500° F. to 700° F. or even higher, at which temperature it may be maintained for a relatively short period of time in order to bring about the desired degree of conversion.

30 When heating or digestion is completed, saponification may be brought about by the addition of caustic soda or other suitable soap forming chemicals to the digested or reacted mixture, preferably without prior cooling of the mixture. On the other hand, cooling may be desirable prior to the addition of the alkaline or basic material depending upon the temperature of the heat reacted mixture, in order to prevent excessive foaming or frothing during its addition.

35 The saponifying agent is preferably added very slowly with continued agitation of the contents of the kettle by the paddles in order to avoid excessive frothing or foaming.

40 Upon completion of saponification the resulting grease preferably is drawn in a molten condition into suitable containers to cool. However, removal of the finished grease from the kettle in a solid or semi-solid condition, as common 45 in the prior art, is not precluded. Likewise the molten grease may be "fibred" by suitable stirring during the initial cooling stages if desired.

45 The following specific examples are given solely for the purpose of illustrating my invention and it is to be understood that I do not intend to limit the invention to the particular proportions, ingredients, or operating conditions recited.

50 In these specific examples the penetration or 55 hardness of the resulting grease is expressed in each instance in terms of tenths of a millimeter penetration of an average sample as determined by the standard A. S. T. M. penetrometer and method for greases, and also with the same apparatus modified to the extent of having an extra weight of 475 grams placed within the penetrometer cone. Such latter reading will be termed "Penetration (Modified ASTM)". This modified 60 penetration test has been used on samples of relatively hard products to penetrate more deeply and give a higher and perhaps more accurate reading than that obtained with the same apparatus without the added weight.

65 A description of the A. S. T. M. penetration test 70 may be found in reports of A. S. T. M. Committee

D-2 on Petroleum Products and Lubricants and Methods of Test Relating to Petroleum Products, under the heading "Tentative Method of Test for Penetration of Greases and Petrolatum," test 75 D-217-27-T.

80

Examples 1, 2 and 3

| Ingredients                                                                                | 1               | 2               | 3                                    | 85    |
|--------------------------------------------------------------------------------------------|-----------------|-----------------|--------------------------------------|-------|
| Cylinder stock (secs. viscosity Saybolt at 210° F.)                                        | 151             | 163             | 220<br>(Distillate)<br>(Cyl. stock.) | 59.20 |
| Per cent.                                                                                  | 37.37           | 39.78           |                                      |       |
| Paraffin distillate (372 secs. viscosity Saybolt at 100° F.) per cent.                     | 22.90           | 24.36           |                                      | 90    |
| Hard tallow per cent.                                                                      | 29.20           | 26.10           | 31.88                                |       |
| Stearic acid per cent.                                                                     | 3.25            | 2.90            |                                      |       |
| Flake caustic (98% NaOH) per cent                                                          | 3.64            | 3.43            | 4.46                                 |       |
| Water, per cent.                                                                           | 3.64            | 3.43            | 4.46                                 |       |
| Time of heating oil and fat mixture before saponification                                  |                 |                 |                                      | 95    |
| Hrs. required to heat to 485° F.                                                           | 5               | 5               | 2                                    |       |
| Hrs. maintained at 485° F.                                                                 | 7               | 11              | 14                                   | 100   |
| Viscosity of mixture (secs. Saybolt at 210° F.)                                            |                 |                 |                                      |       |
| Before heating                                                                             | 70              | 73              | 105                                  |       |
| After heating                                                                              | 104             | 111             | 155                                  | 105   |
| Saponification with caustic soda solution (49% NaOH) consisting of flake caustic and water |                 |                 |                                      |       |
| Hrs. required to add solution                                                              | 4 $\frac{1}{4}$ | 5 $\frac{1}{4}$ | 5 $\frac{1}{2}$                      | 110   |
| Analysis of the final product—per cent. by weight                                          |                 |                 |                                      |       |
| Free alkali                                                                                | Acid.           | Acid.           | 0.28                                 | 115   |
| Water                                                                                      | None.           | None.           | None.                                |       |
| Soda soap                                                                                  | 30.0            | 24.85           | 30.60                                |       |
| Mineral oil                                                                                | 59.95           | 66.22           | 62.54                                |       |
| Free fatty acid (Oleic)                                                                    | 0.42            | 0.42            | 0.14                                 |       |
| Free neutral fat                                                                           | 0.65            | None.           | None.                                |       |
| Undetermined material                                                                      | 8.98            | 8.51            | 6.44                                 |       |
| Physical properties of final product                                                       |                 |                 |                                      | 120   |
| Melting point° F.                                                                          | 370             | 376             | 368                                  |       |
| Penetration (ASTM method)                                                                  | 33              | 29              | 30                                   |       |
| Penetration (modified ASTM)                                                                | 81              | 75              | 75                                   | 125   |

These three examples resulted in relatively hard greases adapted primarily for the lubrication of locomotive driving journals. In Examples 1 and 2 the mineral oil consisted of cylinder stock and 130 a paraffin distillate commonly known in the industry as "heavy red paraffin", the calculated viscosities of the mixed oils being about 90 and 93 seconds, respectively, Saybolt at 210° F. These 135 were heated in admixture with the tallow and stearic acid in the desired proportions to a temperature of about 485° F., and in Example 1 this temperature was maintained for about seven hours while in Example 2 the mixture was maintained at such temperature for a period of about 140 eleven hours. These mixtures when neutralized as nearly as practicable produced greases having nearly the same penetration, Example 2 being slightly harder, while the soap content by 145 actual analysis was at least 5% lower in Example 2 compared with Example 1.

Example 3 shows the use of a heavy distillate cylinder stock having a Saybolt viscosity at 210° F. of 220 seconds which resulted, after heat subjection and neutralization with caustic soda, in a 150

grease showing by analysis 30.6% soda soap and a penetration similar to the other examples.

Obviously, many modifications and variations of the invention as hereinbefore set forth may be made without departing from the spirit and scope thereof, and therefore only such limitations should be imposed as are indicated in the appended claims.

I claim:

- 10 1. A substantially dehydrated lubricating grease adapted for the lubrication of locomotive driving journals, consisting essentially of mineral lubricating oil and between 20 and 35% of soda fatty acid soap, and having a penetration than about 100, and a melting point of about 350 to 400° F.
- 15 2. A substantially dehydrated lubricating grease adapted for the lubrication of locomotive driving journals, consisting essentially of mineral lubricating oil and between 20 and 30% of soda fatty acid soap, and having a penetration

by the modified A. S. T. M. method less than about 100, and a melting point of about 350 to 400° F.

3. A substantially dehydrated lubricating grease adapted for the lubrication of locomotive driving journals, consisting essentially of mineral lubricating oil and about 25% of soda fatty acid soap, and having a penetration by the modified A. S. T. M. method less than about 100, and a melting point of about 350 to 400° F.

4. A substantially dehydrated lubricating grease adapted for the lubrication of locomotive driving journals, consisting essentially of between 20 and 40% of soda fatty acid soap and an oil mixture of cylinder stock and a substantial proportion of a paraffin distillate lubricating oil, said oil mixture having a Saybolt viscosity of less than 125 seconds at 210° F., and having a penetration by the modified A. S. T. M. method less than about 100, and a melting point of about 350 to 400° F.

GUS KAUFMAN.

25

100

30

105

35

110

40

115

45

120

50

125

55

130

60

135

65

140

70

145

75

150